



US010573451B2

(12) **United States Patent**  
**Park et al.**

(10) **Patent No.:** **US 10,573,451 B2**  
(45) **Date of Patent:** **Feb. 25, 2020**

(54) **POWER INDUCTOR**

(71) Applicant: **MODA-INNOCHIPS CO., LTD.**,  
Ansan-Si, Gyeonggi-Do (KR)

(72) Inventors: **In Kil Park**, Seongnam-Si (KR); **Tae Hyung Noh**, Siheung-Si (KR); **Gyeong Tae Kim**, Ansan-Si (KR); **Seung Hun Cho**, Siheung-Si (KR); **Jun Ho Jung**, Sijeung-Si (KR); **Ki Joung Nam**, Siheung-Si (KR); **Jung Gyu Lee**, Seoul (KR)

(73) Assignee: **MODA-INNOCHIPS CO., LTD.** (KR)

(\*) Notice: Subject to any disclaimer, the term of this patent is extended or adjusted under 35 U.S.C. 154(b) by 0 days.

(21) Appl. No.: **15/502,500**

(22) PCT Filed: **Apr. 27, 2015**

(86) PCT No.: **PCT/KR2015/004135**

§ 371 (c)(1),  
(2) Date: **Feb. 7, 2017**

(87) PCT Pub. No.: **WO2016/021807**

PCT Pub. Date: **Feb. 11, 2016**

(65) **Prior Publication Data**

US 2017/0221622 A1 Aug. 3, 2017

(30) **Foreign Application Priority Data**

Aug. 7, 2014 (KR) ..... 10-2014-0101508  
Mar. 9, 2015 (KR) ..... 10-2015-0032400  
Mar. 9, 2015 (KR) ..... 10-2015-0032401

(51) **Int. Cl.**

**H01F 5/00** (2006.01)  
**H01F 27/22** (2006.01)

(Continued)

(52) **U.S. Cl.**

CPC ..... **H01F 27/22** (2013.01); **H01F 17/0013** (2013.01); **H01F 27/255** (2013.01);  
(Continued)

(58) **Field of Classification Search**

USPC ..... 336/200  
See application file for complete search history.

(56) **References Cited**

U.S. PATENT DOCUMENTS

7,497,005 B2 3/2009 Forbes et al.  
9,406,420 B2 \* 8/2016 Ohkubo ..... H01F 5/00  
(Continued)

FOREIGN PATENT DOCUMENTS

CN 1258373 A 6/2000  
CN 101017728 A 8/2007  
(Continued)

OTHER PUBLICATIONS

International Search Report and Written Opinion for PCT/KR2015/004135 dated Jun. 30, 2015.

(Continued)

Primary Examiner — Ronald Hinson

(74) Attorney, Agent, or Firm — Renaissance IP Law Group LLP

(57) **ABSTRACT**

In accordance with an exemplary embodiment, a power inductor includes a body, a base disposed in the body, and a coil pattern disposed on at least one surface of the base, in which the body includes metal powder, a polymer, and a thermal conductive filler and the base is formed by bonding a copper foil to both surfaces of a metal plate comprising iron.

**8 Claims, 4 Drawing Sheets**



|      |                              |                                                                                                                           |                     |              |               |         |
|------|------------------------------|---------------------------------------------------------------------------------------------------------------------------|---------------------|--------------|---------------|---------|
| (51) | <b>Int. Cl.</b>              |                                                                                                                           | JP                  | H11150357 A  | 6/1999        |         |
|      | <i>H01F 27/29</i>            | (2006.01)                                                                                                                 | JP                  | 11260618 A   | 9/1999        |         |
|      | <i>H01F 17/00</i>            | (2006.01)                                                                                                                 | JP                  | 2001057311 A | 2/2001        |         |
|      | <i>H01F 27/255</i>           | (2006.01)                                                                                                                 | JP                  | 2001338813 A | 12/2001       |         |
|      | <i>H01F 27/28</i>            | (2006.01)                                                                                                                 | JP                  | 2002231574 A | 8/2002        |         |
| (52) | <b>U.S. Cl.</b>              |                                                                                                                           | JP                  | 2002305108 A | 10/2002       |         |
|      | CPC .....                    | <i>H01F 27/2804</i> (2013.01); <i>H01F 27/29</i> (2013.01); <i>H01F 27/292</i> (2013.01); <i>H01F 2027/2809</i> (2013.01) | JP                  | 2003059719 A | 2/2003        |         |
|      |                              |                                                                                                                           | JP                  | 2003282328 A | 10/2003       |         |
|      |                              |                                                                                                                           | JP                  | 2003297634 A | 10/2003       |         |
|      |                              |                                                                                                                           | JP                  | 2005038872 A | 2/2005        |         |
|      |                              |                                                                                                                           | JP                  | 2006157738 A | 6/2006        |         |
|      |                              |                                                                                                                           | JP                  | 2006273969 A | 10/2006       |         |
| (56) | <b>References Cited</b>      |                                                                                                                           | JP                  | 2006310812 A | 11/2006       |         |
|      | <b>U.S. PATENT DOCUMENTS</b> |                                                                                                                           | JP                  | 2007012969 A | 1/2007        |         |
|      | 9,899,143 B2                 | 2/2018                                                                                                                    | Kim et al.          | JP           | 2007067214 A  | 3/2007  |
|      | 2002/0105406 A1              | 8/2002                                                                                                                    | Liu et al.          | JP           | 2007194474 A  | 8/2007  |
|      | 2003/0030994 A1              | 2/2003                                                                                                                    | Takaya et al.       | JP           | 2008072073 A  | 3/2008  |
|      | 2005/0080346 A1              | 4/2005                                                                                                                    | Gianchandani et al. | JP           | 2009049335 A  | 3/2009  |
|      | 2007/0080769 A1              | 4/2007                                                                                                                    | Thiel et al.        | JP           | 2009302386 A  | 12/2009 |
|      | 2009/0137067 A1              | 5/2009                                                                                                                    | Forbes et al.       | JP           | 2010010536 A  | 1/2010  |
|      | 2010/0301981 A1              | 12/2010                                                                                                                   | Zeng et al.         | JP           | 2010209469 A  | 9/2010  |
|      | 2011/0007439 A1              | 1/2011                                                                                                                    | Asakawa et al.      | JP           | 2011018756 A  | 1/2011  |
|      | 2011/0178574 A1              | 7/2011                                                                                                                    | Hardy et al.        | JP           | 2011077157 A  | 4/2011  |
|      | 2011/0308072 A1              | 12/2011                                                                                                                   | Ahn et al.          | JP           | 2011258608 A  | 12/2011 |
|      | 2012/0001719 A1*             | 1/2012                                                                                                                    | Oshima .....        | JP           | 2012109292 A  | 6/2012  |
|      |                              |                                                                                                                           |                     | JP           | 2012156461 A  | 8/2012  |
|      |                              |                                                                                                                           |                     | JP           | 2013042102 A  | 2/2013  |
|      |                              |                                                                                                                           |                     | JP           | 20133521414 A | 6/2013  |
|      | 2013/0038417 A1              | 2/2013                                                                                                                    | Kim et al.          | JP           | 2013239542 A  | 11/2013 |
|      | 2013/0082812 A1*             | 4/2013                                                                                                                    | Yoo .....           | JP           | 2014013824 A  | 1/2014  |
|      |                              |                                                                                                                           |                     | JP           | 2014503118 A  | 2/2014  |
|      | 2013/0169401 A1              | 7/2013                                                                                                                    | Lee et al.          | JP           | 5450565 B2    | 3/2014  |
|      | 2013/0222101 A1              | 8/2013                                                                                                                    | Ito et al.          | JP           | 2014110425 A  | 6/2014  |
|      | 2014/0001397 A1              | 1/2014                                                                                                                    | Park et al.         | JP           | 2014130988 A  | 7/2014  |
|      | 2014/0022041 A1              | 1/2014                                                                                                                    | Park et al.         | KR           | 100479625 B1  | 3/2005  |
|      | 2014/0050001 A1              | 2/2014                                                                                                                    | Inaba               | KR           | 20070032259 A | 3/2007  |
|      | 2014/0184374 A1              | 7/2014                                                                                                                    | Park et al.         | KR           | 20120031754 A | 4/2012  |
|      | 2014/0333404 A1*             | 11/2014                                                                                                                   | Bae .....           | KR           | 20120120819 A | 11/2012 |
|      |                              |                                                                                                                           |                     | KR           | 20130046108 A | 5/2013  |
|      |                              |                                                                                                                           |                     | KR           | 20130135298 A | 12/2013 |
|      | 2014/0347773 A1              | 11/2014                                                                                                                   | Park et al.         | KR           | 20140002355 A | 1/2014  |
|      | 2015/0087945 A1              | 3/2015                                                                                                                    | Ziae et al.         | KR           | 20140003056 A | 1/2014  |
|      | 2015/0145627 A1*             | 5/2015                                                                                                                    | Sim .....           | KR           | 20140085997 A | 7/2014  |
|      |                              |                                                                                                                           |                     | TW           | 200915358 A   | 4/2009  |
|      | 2015/0255206 A1*             | 9/2015                                                                                                                    | Han .....           | TW           | 201346951 A   | 11/2013 |
|      |                              |                                                                                                                           |                     | WO           | 2013042691 A1 | 3/2013  |
|      | 2015/0325362 A1              | 11/2015                                                                                                                   | Kumura et al.       | WO           | 2014087888 A1 | 6/2014  |
|      | 2015/0340149 A1*             | 11/2015                                                                                                                   | Lee .....           | JP           | 105K 1/181    | 174/260 |
|      |                              |                                                                                                                           |                     |              |               |         |
|      | 2015/0340150 A1              | 11/2015                                                                                                                   | Nakamura et al.     |              |               |         |

**FOREIGN PATENT DOCUMENTS**

|    |                 |         |
|----|-----------------|---------|
| CN | 101152772 A     | 4/2008  |
| CN | 102969109 A     | 3/2013  |
| CN | 103035354 A     | 4/2013  |
| CN | 103180919 A     | 6/2013  |
| CN | 103578708 A     | 2/2014  |
| CN | 103035354 B     | 11/2016 |
| DE | 102005039379 A1 | 3/2007  |
| JP | H0897045 A      | 4/1996  |
| JP | H08264323 A     | 10/1996 |
| JP | 10241942 A      | 9/1998  |

International Search Report and Written Opinion for PCT/KR2015/005454 dated Aug. 25, 2015.

International Search Report and Written Opinion for PCT/KR2015/008212 dated Nov. 17, 2015.

Office Action for U.S. Appl. No. 15/502,501, dated Jun. 29, 2018.

Office Action for U.S. Appl. No. 15/502,502, dated Jun. 29, 2018.

Extended European Search Report for Application No. 15829073.4 dated May 22, 2018.

Office Action for U.S. Appl. No. 15/502,501, dated May 31, 2019.

\* cited by examiner

FIG. 1



FIG. 2



FIG. 3



FIG. 4



FIG. 5



600 : 610, 620, 630, 640, 650, 660

FIG. 6



FIG. 7



FIG. 8



**1**  
**POWER INDUCTOR**

**BACKGROUND**

The present disclosure relates to a power inductor, and more particularly, to a power inductor having excellent inductance characteristics and improved thermal stability.

A power inductor is generally provided on a power circuit such as a DC-DC converter provided in portable devices. The power inductor is being increasingly used instead of an existing wound type choke coil pattern due to the tendency toward the high frequency and miniaturization of the power circuit. Also, the power inductor is being developed for miniaturization, high current, and low resistance as small-sized and multifunctional the portable devices are required.

The power inductor may be manufactured in the form of a stacked body in which ceramic sheets formed of a plurality of ferrites or a low-k dielectric are stacked. Here, a metal pattern is formed in a coil pattern shape on each of the ceramic sheets. The coil patterns formed on the ceramic sheets are connected to each other by a conductive via formed on each of the ceramic sheets and have a structure in which the coil patterns overlap each other in a vertical direction in which the sheets are stacked. Typically, a body of the power inductor is manufactured by using a magnetic material including a quaternary system of nickel, zinc, copper, and iron.

However, since the magnetic material has a saturation magnetization less than that of a metal material, it may be difficult to realize high current characteristics that are recently required for portable devices. Thus, since the body of the power inductor is formed of metal powder, the saturation magnetization may increase in comparison with a case in which the body is formed of a magnetic material. However, when the body is formed of a metal, a loss of material may increase due to an increase in loss of eddy current and hysteresis in a high frequency. To reduce the loss of the material, a structure in which the metal powder is insulated from each other by using a polymer is being applied.

However, the power inductor including the body formed of the metal powder and polymer may decrease in inductance due to an increase in temperature. That is, the power inductor increases in temperature by heat generated from portable devices to which the power inductor is applied. As a result, while the metal power forming the body of the power inductor is heated, the inductance may decrease.

**PRIOR ART DOCUMENTS**

KR Patent Publication No. 2007-0032259

**SUMMARY**

The present disclosure provides a power inductor which is capable of improving thermal stability to prevent inductance from decreasing.

The present disclosure also provides a power inductor which is capable of releasing heat within a body to improve thermal stability.

In accordance with an exemplary embodiment, a power inductor includes: a body; a base disposed in the body; and a coil pattern disposed on at least one surface of the base, in which the body includes metal powder, a polymer, and a thermal conductive filler.

The metal powder may include metal alloy powder including iron.

**2**

The metal powder may have a surface that is coated with at least one of a magnetic material and insulation material.

The thermal conductive filler may include at least one selected from the group consisting of MgO, AlN, and a carbon-based material.

The thermal conductive filler may be contained in a content of approximately 0.5 wt % to approximately 3 wt %, based on approximately 100 wt % of the metal powder.

10 The thermal conductive filler may have a size of approximately 0.5  $\mu\text{m}$  to approximately 100  $\mu\text{m}$ .

The base may be formed by bonding a copper foil to both surfaces of a metal plate including iron.

15 The power inductor may further include an insulating layer disposed on the coil pattern and an external electrode disposed on an outer portion of the body and connected to the coil pattern.

The power inductor may further include a magnetic layer disposed on at least one area of the body and having 20 magnetic permeability higher than that of the body.

25 The magnetic layer may include the thermal conductive filler.

In accordance with another exemplary embodiment, a power inductor includes: a body; a base disposed in the body; and a coil pattern disposed on at least one surface of the base, in which the base is formed by bonding a copper foil to both surfaces of a metal plate including iron.

30 The body may include metal powder, a polymer, and a thermal conductive filler.

35 The thermal conductive filler may include at least one selected from the group consisting of MgO, AlN, and a carbon-based material.

The thermal conductive filler may be contained in a content of approximately 0.5 wt % to approximately 3 wt %, based on approximately 100 wt % of the metal powder.

40 The power inductor may further include an insulating layer disposed on at least one area of the body and having magnetic permeability higher than that of the body.

**Advantageous Effects**

In the power inductor according to the embodiments of the present invention, the body may be manufactured by the metal powder, the polymer, and the thermal conductive filler.

45 The thermal conductive filler may be provided to well release the heat of the body to the outside, and thus, the reduction of the inductance due to the heating of the body may be prevented.

Also, the base material that is provided inside the body 50 and on which the coil pattern is formed may be manufactured by using the metal magnetic material to prevent the power inductor from being deteriorated in magnetic permeability. In addition, at least one magnetic layer may be disposed on the body to improve the magnetic permeability of the power inductor.

**BRIEF DESCRIPTION OF THE DRAWINGS**

Exemplary embodiments can be understood in more detail 60 from the following description taken in conjunction with the accompanying drawings, in which:

FIG. 1 is a perspective view of a power inductor in accordance with an exemplary embodiment;

FIG. 2 is a cross-sectional view taken along line A-A' of 65 FIG. 1;

FIGS. 3 to 5 are cross-sectional views of a power inductor in accordance with other exemplary embodiments; and

FIGS. 6 to 8 are cross-sectional views for explaining a method for manufacturing the power inductor in accordance with an exemplary embodiment.

#### DETAILED DESCRIPTION OF EMBODIMENTS

Hereinafter, specific embodiments will be described in detail with reference to the accompanying drawings. The present disclosure may, however, be embodied in many different forms and should not be construed as being limited to the embodiments set forth herein. Rather, these embodiments are provided so that this disclosure will be thorough and complete, and will fully convey the concept of the invention to those skilled in the art.

FIG. 1 is a perspective view of a power inductor in accordance with an exemplary embodiment, and FIG. 2 is a cross-sectional view taken along line A-A' of FIG. 1.

Referring to FIGS. 1 and 2, a power inductor in accordance with an exemplary embodiment may include a body 100 including a thermal conductive filler 130, a base 200 provided in the body 100, coil patterns 310 and 320 disposed on at least one surface of the base 200, and external electrodes 410 and 420 disposed outside the body 100.

The body 100 may have, for example, a hexahedral shape. The body 100, however, may have a polyhedral shape in addition to the hexahedral shape. The body 100 may include metal powder 110, a polymer 120, and a thermal conductive filler 130. The metal powder 110 may have a mean particle diameter of approximately 1  $\mu\text{m}$  to approximately 50  $\mu\text{m}$ . Also, the metal powder 110 may use a single kind of or at least two kinds of particles having the same size and a single kind of or at least two kinds of particles having a plurality of sizes. For example, a first metal particle having a mean size of approximately 30  $\mu\text{m}$  and a second metal particle having a mean size of approximately 3  $\mu\text{m}$  may be mixed with each other for using. When at least two kinds of metal powder 110 having sizes different from each other are used, the body 100 may increase in filling rate to maximize capacity. For example, when metal powder having a size of approximately 30  $\mu\text{m}$  is used, a pore may be generated between the metal powder having the size of approximately 30  $\mu\text{m}$ , resulting in decreasing the filling rate. However, since metal power having a size of approximately 3  $\mu\text{m}$  is mixed between the metal power having the size of approximately 30  $\mu\text{m}$ , the filling rate may further increase. The metal powder 110 may use a metal material including iron (Fe). For example, the metal powder 110 may include at least one metal selected from the group consisting of iron-nickel (Fe—Ni), iron-nickel-silica (Fe—Ni—Si), iron-aluminum-silica (Fe—Al—Si), and iron-aluminum-chrome (Fe—Al—Cr). That is, since the metal powder 110 includes the iron, the metal powder 110 may be formed as a metal alloy having a magnetic structure or magnetic property to have predetermined magnetic permeability. Also, surface of the metal powder 110 may be coated with a magnetic material having magnetic permeability different from that of the metal powder 110. For example, the magnetic material may be formed of a metal oxide magnetic material. That is, the magnetic material may be formed of at least one oxide magnetic material selected from the group consisting of a nickel-oxide magnetic material, a zinc-oxide magnetic material, a copper-oxide magnetic material, a manganese-oxide magnetic material, a cobalt-oxide magnetic material, a barium-oxide magnetic material, and a nickel-zinc-copper oxide magnetic material. The magnetic material applied on the surface of the metal powder 110 may be formed of a metal oxide including iron and have the magnetic perme-

ability greater than that of the metal powder 110. Furthermore, the surface of the metal powder 110 may be coated with at least one insulation material. For example, the surface of the metal powder 110 may be coated with an oxide and an insulating polymer material such as parylene. The oxide may be formed by oxidizing the metal powder 110 or be coated with one selected from the group consisting of TiO<sub>2</sub>, SiO<sub>2</sub>, ZrO<sub>2</sub>, SnO<sub>2</sub>, NiO, ZnO, CuO, CoO, MnO, MgO, Al<sub>2</sub>O<sub>3</sub>, Cr<sub>2</sub>O<sub>3</sub>, Fe<sub>2</sub>O<sub>3</sub>, B<sub>2</sub>O<sub>3</sub>, and Bi<sub>2</sub>O<sub>3</sub>. Also, the surface of the metal powder 110 may be coated by using various insulating polymer materials in addition to the parylene. Here, the metal powder 110 may be coated with oxide having a double-layered structure or a double-layered structure of oxide and polymer materials. Alternatively, the surface of the metal powder 110 may be coated with the magnetic material and then the insulating material. As described above, the surface of the metal powder 110 may be coated with the insulating material to prevent a short-circuit due to the contact of the metal powder 110 from occurring. The polymer 120 may be mixed with the metal powder 110 so that the metal powder 110 is insulated with each other. That is, the metal powder 110 may increase in loss of eddy current and hysteresis in a high frequency to cause a loss of the material. To reduce the loss of the material, the polymer 120 may be provided to insulate the metal powder 110 from each other. Although the polymer 120 is selected from the group consisting of epoxy, polyimide, and a liquid crystalline polymer (LCP), the present disclosure is not limited thereto. Also, the polymer 120 may include a thermosetting resin to give an insulation property to the metal powder 110. The thermosetting resin may include at least one selected from the group consisting of a novolac epoxy resin, a phenoxy type epoxy resin, a BPA type epoxy resin, a BPF type epoxy resin, a hydrogenated BPA epoxy resin, a dimer acid modified epoxy resin, a urethane modified epoxy resin, a rubber modified epoxy resin, and a DCPD type epoxy resin. Here, the polymer 120 may be contained in a content of approximately 2.0 wt % to approximately 5.0 wt %, based on 100 wt % of the metal powder. When the polymer 120 increases in content, a volume fraction of the metal powder 110 may decrease, and thus, it may be difficult to properly realize an effect for increasing the saturation magnetization, and the magnetic characteristics of the body 100, i.e., the magnetic permeability may decrease. When the polymer 120 decreases in content, a strong acid or strong alkaline solution used in a process for manufacturing the inductor may be permeated into the inductor to reduce the inductance characteristics. Thus, the polymer 120 may be contained within a range in which the saturation magnetization and inductance of the metal powder 110 do not decrease. Also, the thermal conductive filler 130 may be provided to solve the limitation in which the body 100 is heated by the external heat. That is, when the metal powder 110 of the body 100 is heated by the external heat, the thermal conductive filler 130 may release the heat of the metal powder 110 to the outside. Although the thermal conductive filler 130 includes at least one selected from the group consisting of MgO, AlN, and a carbon-based material, the present disclosure is not limited thereto. Here, the carbon-based material may include carbon and have various shapes. For example, the carbon-based material may include graphite, carbon black, graphene, graphite, and the like. Also, the thermal conductive filler 130 may be contained in a content of approximately 0.5 wt % to approximately 3 wt %, based on approximately 100 wt % of the metal powder 110. When the content of the thermal conductive filler 130 is below the above-described range, a heat dissipation effect

may not be achieved. On the other hand, when the content of the thermal conductive filler 130 is above the above-described range, the magnetic permeability of the metal powder 110 may decrease. Also, the thermal conductive filler 130 may have, for example, a size of approximately 0.5  $\mu\text{m}$  to approximately 100  $\mu\text{m}$ . That is, the thermal conductive filler 130 may have a size greater or less than that of the metal powder 110. On the other hand, the body 100 may be manufactured by stacking a plurality of sheets formed of a material including the metal powder 110, the polymer 120, and the thermal conductive filler 130. Here, when the body 100 is manufactured by stacking the plurality of sheets, the thermal conductive fillers 130 in the sheets may have contents different from each other. For example, the more the thermal filters are away from the base 200 upward and downward, the content of the thermal conductive fillers 130 in the sheets may gradually increase in content. Also, as necessary, the body 100 may be formed by applying various processes such as a process of printing paste formed of a material including the metal powder 110, the polymer 120, and the thermal conductive filler 130 at a predetermined thickness or a process of filling the paste into a frame to compress the paste. Here, the number of sheets stacked for forming the body 100 or a thickness of the paste printed at the predetermined thickness may be determined to adequate number or thickness in consideration of electrical characteristics such as the inductance required for the power inductor.

The base 200 may be provided in the body 100. At least one base 200 may be provided. For example, the base 200 may be provided in the body 100 in a longitudinal direction of the body 100. Here, at least one base 200 may be provided. For example, two bases 200 may be provided in a direction perpendicular to a direction in which the external electrode 400 is disposed, for example, be spaced a predetermined distance from each other in a vertical direction. The base 200, for example, may be formed of copper clad lamination (CCL), a metal magnetic material, or the like. Here, the base 200 is formed of the magnetic material to improve the magnetic permeability and easily realize the capacity. That is, the CCL is manufactured by bonding a copper foil to glass reinforced fiber. Thus, the CCL may not have the magnetic permeability to reduce the magnetic permeability of the power inductor. However, when the metal magnetic material is used as the base 200, the magnetic permeability of the power inductor may not be reduced because the metal magnetic material has the magnetic permeability. The base 200 using the metal magnetic material may be manufactured by bonding the copper foil to a plate that has a predetermined thickness and is formed of at least one metal selected from the group consisting of metal including iron such as, for example, iron-nickel (Fe—Ni), iron-nickel-silica (Fe—Ni—Si), iron-aluminum-silica (Fe—Al—Si), and iron-aluminum-chrome (Fe—Al—Cr). That is, an alloy formed of at least one metal including iron may be manufactured in the form of a plate having a predetermined thickness, and then the copper foil may be bonded to at least one surface of the metal plate to manufacture the base 200. Also, at least one conductive via (not shown) may be formed in a predetermined area of the base 200, and the coil patterns 310 and 320 respectively disposed on the upper and lower portions of the base 200 may be electrically connected to each other by the conductive via. The via (not shown) passing in a thickness of the base 200 may be formed, and then the conductive paste may be filled into the via to form the conductive via.

The coil patterns 310 and 320 may be disposed on at least one surface, preferably, both surfaces of the base 200. The coil patterns 310 and 320 may be disposed on a predetermined area of the base 200, e.g., disposed outward from a central portion thereof in a spiral shape, and the two coil patterns 310 and 320 disposed on the base 200 may be connected to form one coil. Here, the coil patterns 310 and 320 on the upper and lower portions may have the same shape. Also, the coil patterns 310 and 320 may overlap each other. Alternatively, the coil pattern 320 may overlap each other on an area in which the coil pattern 310 is not formed. The coil patterns 310 and 320 may be electrically connected by the conductive via formed in the base 200. The coil patterns 310 and 320 may be formed by a method such as, for example, screen printing, coating, deposition, plating, or sputtering. Although each of the coil patterns 310 and 320 and the conductive via is formed of a material including at least one of silver (Ag), copper (Cu), and copper alloy, the present disclosure is not limited thereto. On the other hand, when the coil patterns 310 and 320 are formed through the plating process, the metal layer, for example, a copper layer may be formed on the base 200 by the plating process and then be patterned by a lithography process. That is, the copper layer may be formed by using the copper foil as a seed layer through the plating process and then be patterned to form the coil patterns 310 and 320. Alternatively, a photosensitive film pattern having a predetermined shape may be formed on the base 200, and the plating process may be performed to grow the metal layer from the exposed surface of the base 200, and then the photosensitive film may be removed to form the coil patterns 310 and 320 having a predetermined shape. Alternatively, the coil patterns 310 and 320 may be formed in a multi-layered shape. That is, a plurality of coil patterns may be further formed upward from the coil patterns 310 formed on the upper portion of the base 200, and a plurality of coil patterns may be further formed downward from the coil patterns 320 formed on the lower portion of the base 200. When the coil patterns 310 and 320 are formed in the multi-layered shape, an insulation layer may be formed between lower and upper layers, and a conductive via (not shown) may be formed in the insulation layer to connect the multi-layered coil patterns to each other.

The external electrodes 400 may be formed on both ends of the body 100, respectively. For example, the external electrodes 400 may be formed on both side surfaces facing each other in the longitudinal direction of the body 100. The external electrodes 400 may be electrically connected to the coil patterns 310 and 320 of the body 100. That is, at least one end of the coil patterns 310 and 320 may be exposed to the outside, and the external electrode 400 may be connected to the exposed end of the coil patterns 310 and 320. The external electrodes 400 may be formed on both ends of the body 100 by dipping the body 100 into the conductive paste or through the various processes such as the printing, the deposition, and the sputtering. The external electrode 400 may be formed of an electro-conductive metal that is selected from the group consisting of gold, silver, platinum, copper, nickel, palladium, and an alloy thereof. Also, a nickel-plated layer (not shown) or a tin-plated layer (not shown) may be further formed on a surface of the external electrode 400.

Alternatively, an insulation layer 500 may be further formed between the coil patterns 310 and 320 and the body 100 to insulate the coil patterns 310 and 320 from the metal powder 110. That is, the insulation layer 500 may be formed on the upper and lower portions of the base 200 to cover the coil patterns 310 and 320. The insulation layer 500 may

include at least one material selected from the group consisting of epoxy, polyimide, and a liquid crystal crystalline polymer. That is, the insulation layer **500** may be formed of the same material as the polymer **120** forming the body **100**. Also, the insulation layer **500** may be formed by applying an insulating polymer material such as parylene on the coil patterns **310** and **320**. That is, the insulation layer **500** may be coated at a uniform thickness along stepped portions of the coil patterns **310** and **320**. Alternatively, the insulation layer **500** may be formed on the coil patterns **310** and **320** by using the insulation sheet.

As above-described, the power inductor in accordance with an exemplary embodiment may include the body **100** including the metal powder **110**, the polymer **120**, and the thermal conductive filler **130**. The thermal conductive filler **130** may be provided in the body **100** to release the heat of the body **100**, which is generated by heating of the metal powder **110**, to the outside, thereby preventing the body **100** from increasing in temperature, and thus, preventing the inductance from being reduced. Also, the base **200** inside the body **100** may be formed of the magnetic material to prevent the power inductor from being reduced in magnetic permeability.

FIG. 3 is a cross-sectional view of a power inductor in accordance with another exemplary embodiment.

Referring to FIG. 3, a power inductor in accordance with another exemplary embodiment may include a body **100** including a thermal conductive filler **130**, a base **200** provided in the body **100**, coil patterns **310** and **320** disposed on at least one surface of the base **200**, external electrodes **410** and **420** disposed outside the body **100**, and at least one magnetic layer **600** (**610** and **620**) respectively provided on upper and lower portions of the body **100**. Also, the power inductor may further include an insulation layer **500** provided on each of the coil patterns **310** and **320**. That is, the magnetic layer **600** may be further provided in the power inductor in accordance with an embodiment to realize another embodiment. Another embodiment will be described below regarding constitutions different from the foregoing embodiment.

A magnetic layer **600** (**610** and **620**) may be provided to at least one area of a body **100**. That is, a first magnetic layer **610** may be disposed on a top surface of the body **100**, and a second magnetic layer **620** may be disposed on a bottom surface of the body **100**. Here, the first and second magnetic layers **610** and **620** may be provided to increase magnetic permeability of the body **100** and be formed of a material having magnetic permeability higher than that of the body **100**. For example, the body **100** may have magnetic permeability of approximately 20, and each of the first and second magnetic layers **610** and **620** may have magnetic permeability of approximately 40 to approximately 1000. The first and second magnetic layers **610** and **620** may be formed of, for example, magnetic powder and a polymer. That is, the first and second magnetic layers **610** and **620** may be formed of a material having magnetism higher than that of the magnetic material of the body **100** or have a content of the magnetic material, which is higher than that of the magnetic material of the body **100** so that each of the first and second magnetic layers **610** and **620** has the magnetic permeability higher than that of the body **100**. Here, the polymer may be contained in a content of approximately 15 wt %, based on approximately 100 wt % of the metal powder. Also, the magnetic material powder may use at least one selected from the group consisting of a nickel magnetic material (Ni Ferrite), a zinc magnetic material (Zn Ferrite), a copper magnetic material (Cu Ferrite), a manganese magnetic mate-

rial (Mn Ferrite), a cobalt magnetic material (Co Ferrite), a barium magnetic material (Ba Ferrite), and a nickel-zinc-copper magnetic material (Ni—Zn—Cu Ferrite) or at least one oxide magnetic material thereof. That is, the magnetic layer **600** may be formed by using a metal alloy powder including iron or a metal alloy oxide including iron. Also, the magnetic powder may be formed by applying the magnetic material to the metal alloy powder. For example, the magnetic material powder may be formed by applying at least one magnetic material oxide selected from the group consisting of a nickel-oxide magnetic material, a zinc-oxide magnetic material, a copper-oxide magnetic material, a manganese-oxide magnetic material, a cobalt-oxide magnetic material, a barium-oxide magnetic material, and a nickel-zinc-copper oxide magnetic material to, for example, the metal alloy powder including iron. That is, the magnetic material powder may be formed by applying the metal oxide including iron to the metal alloy powder. Alternatively, the magnetic material powder may be formed by mixing at least one magnetic material oxide selected from the group consisting of a nickel-oxide magnetic material, a zinc-oxide magnetic material, a copper-oxide magnetic material, a manganese-oxide magnetic material, a cobalt-oxide magnetic material, a barium-oxide magnetic material, and a nickel-zinc-copper oxide magnetic material with, for example, the metal alloy powder including iron. That is, the magnetic material powder may be formed by mixing the metal oxide including iron with the metal alloy powder. On the other hand, each of the first and second magnetic layers **610** and **620** may further include the thermal conductive fillers in addition to the metal powder and polymer. The thermal conductive fillers may be contained in a content of approximately 0.5 wt % to approximately 3 wt %, based on approximately 100 wt % of the metal powder. The first and second magnetic layers **610** and **620** may be manufactured in a sheet shape and respectively disposed on upper and lower portions of the body **100** on which a plurality of sheets are stacked. Also, the body **100** may be formed by printing a paste formed of a material including metal powder **110**, a polymer **120**, and a thermal conductive filler **130** at a predetermined thickness or filling the paste into a frame to compress the paste, and then the magnetic layer **610** and **620** may be respectively disposed on the upper and lower portions of the body **100**. Alternatively, the magnetic layer **610** and **620** may be formed by using the paste, i.e., formed by applying the magnetic material to the upper and lower portions of the body **100**.

The power inductor in accordance with an exemplary embodiment may further include third and fourth magnetic layers **630** and **640** on the upper and lower portions between the body **100** and the base **200** as illustrated in FIG. 4, and fifth and sixth magnetic layers **650** and **660** may be further provided therebetween as illustrated in FIG. 5. That is, at least one magnetic layer **600** may be provided in the body **100**. The magnetic layers **600** may be manufactured in a sheet shape and provided in the body **100** in which a plurality of sheet are stacked. That is, at least one magnetic layer **600** may be provided between the plurality of sheets for manufacturing the body **100**. Also, when the body **100** is formed by printing the paste formed of the material including the metal powder **110**, the polymer **120**, and the thermal conductive filler **130** at a predetermined thickness, the magnetic layer may be formed during the printing. Also, when the body **100** is formed by filling the paste into the frame to compress the paste, the magnetic layer may be inserted therebetween to compress the paste. Alternatively, the magnetic layer **600** may be formed by using the paste,

i.e., formed in the body 100 by applying a soft magnetic material during the printing of the body 100.

As described above, the power inductor in accordance with another exemplary embodiment may include the at least one magnetic layer 600 in the body 100 to improve the magnetism of the power inductor.

FIGS. 6 to 8 are cross-sectional views sequentially illustrating a method for manufacturing the power inductor in accordance with an exemplary embodiment.

Referring to FIG. 6, coil patterns 310 and 320 each of which has a predetermined shape are formed on at least one surface, preferably, both surfaces of a base 200. The base 200 may be formed of CCL, a metal magnetic material, or the like. For example, the base 200 may be formed of a metal magnetic material that is capable of improving effective magnetism and easily realizing capacity. For example, the base 200 may be manufactured by bonding a copper foil to both surfaces of a metal plate which is formed of a metal alloy including iron and has a predetermined thickness. Also, the coil patterns 310 and 320 may be formed on a predetermined area of the base 200, e.g., may be formed as a coil pattern that is formed from a central portion thereof in a circular spiral shape. Here, the coil pattern 310 may be formed on one surface of the base 200, and then a conductive via passing through a predetermined area of the base 200 and in which a conductive material is filled therein may be formed. Also, the coil pattern 320 may be formed on the other surface of the base 200. The conductive via may be formed by filling conductive paste into a via hole after the via hole is formed in a thickness direction of the base 200 by using laser. For example, the coil pattern 310 may be formed through a plating process. For this, a photosensitive pattern having a predetermined shape may be formed on one surface of the base 200 to perform the plating process using a copper foil as a seed on the base 200. Then, a metal layer may be grown from the exposed surface of the base 200, and then the photosensitive film may be removed. Alternatively, the coil patterns 320 may be formed on the other surface of the base 200 by using the same manner as that for forming the coil pattern 310. Alternatively, the coil patterns 310 and 320 may be formed in a multi-layered shape. When the coil patterns 310 and 320 are formed in the multi-layered shape, an insulation layer may be formed between lower and upper layers, and the conductive via (not shown) may be formed in the insulation layer to connect the multi-layered coil patterns to each other. The coil patterns 310 and 320 are formed on one surface and the other surface of the base 200, respectively, and then the insulation layer 500 is formed to cover the coil patterns 310 and 320. The insulation layer 500 may be formed by closely attaching a sheet including at least one material selected from the group consisting of epoxy, polyimide, and a liquid crystal crystalline polymer to the coil patterns 310 and 320.

Referring to FIG. 7, a plurality of sheets 100a to 100h formed of a material including the metal powder 110, the polymer 120, and the thermal conductive filler 130 are provided. Here, the metal powder 110 may use a metal material including iron (Fe), and the polymer 120 may use epoxy, polyimide, or the like, which is capable of insulating the metal powder 110 from each other. Also, the thermal conductive filler 130 may use MgO, AlN, a carbon based material, or the like, which is capable of releasing heat of the metal powder 110 to the outside. Also, the surface of the metal powder 110 may be coated with a magnetic material, for example, a metal oxide magnetic material. Here, the polymer 120 may be contained in a content of approximately 2.0 wt % to approximately 5.0 wt %, based on 100 wt % of

the metal powder 110, and the thermal conductive fillers 130 may be contained in a content of approximately 0.5 wt % to approximately 3.0 wt %, based on 100 wt % of the metal powder 110. The plurality of sheets 100a to 100h are disposed on the upper and lower portions of the base 200 on which the coil patterns 310 and 320 are formed, respectively. Here, the plurality of sheets 100a to 100h may have contents of thermal conductive fillers 130, which are different from each other. For example, the thermal conductive fillers 130 may have contents that gradually increase from one surface and the other surface of the base 200 toward the upper and lower sides of the base 200. That is, the thermal conductive filters 130 of the sheets 100b and 100e disposed on upper and lower portions of the sheets 100a and 100d contacting the base 200 may have contents higher than those of the thermal conductive filters 130 of the sheets 100a and 100d, and the thermal conductive filters 130 of the sheets 100c and 100f disposed on upper and lower portions of the sheets 100b and 100e may have contents higher than those of the thermal conductive filters 130 of the sheets 100b and 100e. Like this, the contents of the thermal conductive fillers 130 may gradually increase in a direction that is away from the base 200 to further improve heat transfer efficiency. As described in another exemplary embodiment, the first and second magnetic layers 610 and 620 may be provided to the upper and lower portions of the uppermost and lowermost sheets 100a and 100h, respectively. Each of the first and second magnetic layers 610 and 620 may be formed of a material having magnetic permeability higher than that of each of the sheets 100a to 100h. For example, each of the first and second magnetic layers 610 and 620 may be formed of magnetic powder and an epoxy resin so that each of the first and second magnetic layers 610 and 620 has magnetic permeability higher than that of each of the sheets 100a to 100h. Also, each of the first and second magnetic layers 610 and 620 may further include the thermal conductive fillers.

Referring to FIG. 8, the plurality of sheets 100a to 100h are stacked and compressed with the base 200 therebetween and then molded to form the body 100. The external electrodes 400 may be formed so that the protruding portion of each of the coil patterns 310 and 320 is electrically connected to both ends of the body 100. The external electrodes 400 may be formed by various processes including a process of dipping the body 100 into a conductive paste, a process of printing the conductive past on both ends of the body 100, a deposition process, and a sputtering process. Here, the conductive paste may use a metal material that is capable of giving electric conductivity to the external electrode 400. Also, a nickel plated layer and a tin plated layer may be further formed on a surface of the external electrode 400, if necessary.

In accordance with the exemplary embodiments, the body of the power inductor may be formed of the metal powder, the polymer, and the thermal conductive filler. Since the thermal conductive filler is provided, the heat in the body may be easily released to the outside to prevent the inductance from decreasing due to the heated body.

Also, the base, on which the coil pattern is formed, disposed in the body may be formed of the metal magnetic material to prevent the magnetic permeability of the power inductor from decreasing, and the at least one magnetic layer may be provided on the body to improve the magnetic permeability of the power inductor.

The power inductor may not be limited to the foregoing embodiments, but be realized through various embodiments different from each other. Therefore, it will be readily understood by those skilled in the art that various modifi-

**11**

cations and changes can be made thereto without departing from the spirit and scope of the present invention defined by the appended claims.

What is claimed is:

1. A power inductor comprising:

a body;

a base disposed in the body; and

a coil pattern disposed on at least one surface of the base, wherein the body comprises a metal powder, a polymer, and a thermal conductive filler particle for discharging

heat of the metal powder to the outside,

wherein only the metal powder comprises a metal magnetic material,

wherein the thermal conductive filler particle has a size of approximately 0.5  $\mu\text{m}$  to approximately 100  $\mu\text{m}$ , and wherein the thermal conductive filler particle is dispersed in the polymer, made from a different material from the polymer, and contained in a content of approximately 0.5 wt % to approximately 3 wt %, based on approximately 100 wt % of the metal powder.

**12**

2. The power inductor of claim 1, wherein the thermal conductive filler particle comprises at least one selected from the group consisting of MgO, AlN, and a carbon-based material.

5 3. The power inductor of claim 1, wherein the base is formed by bonding a copper foil to both surfaces of a metal plate comprising iron.

4. The power inductor of claim 1, further comprising an insulating layer disposed on the coil pattern and an external electrode disposed on an outer portion of the body and connected to the coil pattern.

5. The power inductor of claim 1, wherein the metal powder comprises metal alloy powder comprising iron.

6. The power inductor of claim 5, wherein the metal powder has a surface that is coated with at least one of a magnetic material and insulation material.

7. The power inductor of claim 1, further comprising a magnetic layer disposed on at least one area of the body and having magnetic permeability higher than that of the body.

20 8. The power inductor of claim 7, wherein the magnetic layer comprises the thermal conductive filler particle.

\* \* \* \* \*